

M. D. WILBUR, F. P. CANNON AND T. J. MURPHY,  
PROCESS FOR CARBONIZING ARTICLES AND APPARATUS FOR SAME.  
APPLICATION FILED JULY 26, 1917.

1,350,483.

Patented Aug. 24, 1920.

2 SHEETS—SHEET 1.



Fig. 1.



Fig. 2.



Fig. 3.

INVENTORS.

Mark D. Wilbur  
Frederick P. Cannon  
BY Thomas J. Murphy  
Parsons & Borrell  
ATTORNEYS

M. D. WILBUR, F. P. CANNON AND T. J. MURPHY,  
PROCESS FOR CARBONIZING ARTICLES AND APPARATUS FOR SAME.  
APPLICATION FILED JULY 26, 1917.

1,350,483.

Patented Aug. 24, 1920.

2 SHEETS—SHEET 2.



Fig. 4.



Fig. 5.

INVENTORS.  
Maurit D. Wilbur  
Francis P. Cannon  
BY Thomas J. Murphy  
Parsons, Brinckerhoff,  
ATTORNEYS.

# UNITED STATES PATENT OFFICE.

MERRITT D. WILBUR, OF ROCHESTER, FRANCIS P. CANNON, OF SYRACUSE, AND  
THOMAS J. MURPHY, OF ROCHESTER, NEW YORK.

## PROCESS FOR CARBONIZING ARTICLES AND APPARATUS FOR SAME.

1,350,483.

Specification of Letters Patent. Patented Aug. 24, 1920.

Application filed July 26, 1917. Serial No. 182,926.

To all whom it may concern:

Be it known that we, MERRITT D. WILBUR, FRANCIS P. CANNON, citizens of the United States, and residents of Rochester, in the 5 county of Monroe and State of New York, and of Syracuse, in the county of Onondaga and State of New York, respectively, and THOMAS J. MURPHY, a citizen of the Dominion of Canada, and a resident of Rochester, 10 in the county of Monroe and State of New York, have invented a certain new and useful Process for Carbonizing Articles and Apparatus for Same, of which the following is a specification.

15 This invention has for its object an apparatus and process of carbonizing articles, especially ferrous articles by applying quickly generated heat, as electrically generated heat, and thereby quickly raising the 20 temperature of the articles and the carbonizing material above the critical point so that the carbonizing is accomplished in a relatively short time as compared with several hours by other processes. The invention 25 consists in the steps and operations and the apparatus hereinafter set forth and claimed.

In describing this invention, reference is had to the accompanying drawings in which like characters designate corresponding 30 parts in all the views.

Figures 1, 2 and 3 are diagrammatical views of different forms of apparatus for carrying out our process and different ways of subjecting the articles to electrically generated heat.

Fig. 4 is a plan view partly broken away, of one form of the apparatus shown in Fig. 1.

Fig. 5 is a sectional view on line 5—5, 40 Fig. 4.

This process of carbonizing articles, as ferrous articles, consists in surrounding the article or articles with a carbonizing material, quickly raising the temperature of 45 such material and the articles above the critical point, and maintaining the temperature at the desired point for the required length of time depending on the depth it is desired to cement or to carbonize. The material is generally packed and subjected to 50 substantial mechanical pressure and the heat is preferably electrically generated heat. By the expression "electrically generated heat" is meant heat generated by the resistance of the carbonizing material to an electric current passing therethrough, or heat

generated by the resistance of an electric heat unit, as a grid, around which the carbonizing medium is placed and from which it receives heat by conduction, or heat generated by an induced current generated in the carbonizing material and the ferrous articles by the alternating magnetic flux. 60

In operation, the articles are packed in the carbonizing material, which may be 65 pulverized bone dust, or carbonized oils in the form of small pellets, and the carbonized material heated. The heat is brought quickly to the desired temperature preferably above the critical point, ordinarily from 1600° to 70 1800° F. more or less, depending somewhat on the structure and the size of the articles being treated.

It is believed that the electric current either passing directly through the carbonizing material and articles being heated or generated or induced therein, facilitates the carbonizing process, and renders the product more satisfactory in that it has a direct influence other than the mere generation of 80 heat.

The electrically generated heat may be utilized conductively, convectively or inductively, in accordance with the apparatus employed. 85

The apparatus shown in Fig. 1, comprises a container having a lining 1 of fire clay or some non-conductive and highly refractory material, and electrodes 2, 3 exposed in the container on opposite sides thereof and between which are placed the articles 4 to be carbonized, and any improved carbonizing material 5 such as bone dust or carbonized oil. The electrodes are connected in an electric circuit, usually of low potential and high amperage, which tends toward uniformity of heat distribution. Preferably, substantial mechanical pressure is also applied to compress the carbonizing material as applying mechanical pressure to the carbon particles makes the mass a conductor, as a whole, and hence the current cannot localize in any one path but must distribute itself throughout the mass. By applying pressure, it is possible to use a low voltage 105 current of high amperage, and also render the carbonizing material a homogeneous conducting mass. By using a current of low voltage great economy in operation is effected compared with the processes and apparatus using high voltage or an electric arc. 110

In the operation of this apparatus, the

carbonizing material rises rapidly in temperature owing to its resistance to the electric current, and heats directly by conduction the surfaces of the articles to be carbonized.

The apparatus shown in Fig. 2 comprises a suitable container having a lining 6 of refractory and non-conductive material and a heating unit or grid 7 located in the container and capable of withstanding a high temperature and offering high resistance to the passage of electric current, the grid being connected in an electric circuit.

In operation, the articles 8 to be carbonized are placed in suitable proximity to the grid and then the carbonizing material 9 is packed around the articles, it being understood that initially a layer of carbonizing material is placed in the container and then one or more articles arranged upon this layer and the container filled with layers of articles and carbonizing material, care being taken to have the articles and the grid entirely surrounded by the packing material.

In this method of carrying out our process, it is not necessary that the carbonizing material be subjected to mechanical pressure, but on the contrary for some purposes it is preferable not to use pressure. The grid, owing to the resistance it offers to the electrical current, becomes heated and heats the carbonizing material by conduction, which in turn heats directly the surfaces of the articles being carbonized.

The apparatus shown in Fig. 3 comprises a laminated core or electromagnet 10 forming a closed magnetic circuit, the core being energized by primary windings 11 connected in the electrical circuit, and containers 12 of refractory and nonconducting material inclosing portions of the core. The articles 4<sup>a</sup> are packed around or caused to encircle the portions of the laminated core in the containers, the carbonizing material 5<sup>a</sup> is then packed around the articles within the container and usually subjected to mechanical pressure. It is not, however, necessary or essential that the articles to be carbonized encircle a part of the core 10 as they may be satisfactorily treated within the container even though not encircling the core, owing to the fact that the increased temperature brought about in the conductive packing material is effective conductively on such articles. The refractory containers 12 are lined with graphite cylinders 12<sup>a</sup> and concentric graphite rings 12<sup>b</sup> may be distributed in the pellets. In operation, the magnetic flux induces a secondary current in the articles in the container, and also in the packing material, and, owing to the resistance offered to the current by the packing material, heat is generated.

The apparatus set forth herein are merely

illustrative of various means of carrying out our process, and it will be understood by those skilled in the art that our process is not limited to any particular construction of apparatus.

In any of the instances, the heat applied 70 is electrically generated. In the form shown in Fig. 1, the heat is generated by the current passing between the electrodes 2, 3 through the carbonizing material, and the heat is applied conductively to the surface 75 of the articles being treated. In the form shown in Fig. 2, the heat is electrically generated in the heating unit or grid 7, and transferred conductively to the carbonizing material, and by the heated carbonizing material to the surfaces of the article being treated.

In the form shown in Fig. 3, the heat is generated in the carbonizing material 5<sup>a</sup> by the induced current generated by the alternating magnetic flux through the laminated core.

In both the forms shown in Figs. 1 and 3, the current passes through the carbonizing material and also through the article being treated, and the presence of this current passing through the article in the carbonizing process tends to render the product more satisfactory.

In Figs. 4 and 5, we have illustrated one 95 form of apparatus shown diagrammatically in Fig. 1, the apparatus shown in Fig. 4 being constructed to facilitate the even distribution of the current and the resultant heat through the carbonizer, especially 100 where the apparatus is of considerable length for treating long pieces of ferrous parts through which it is preferable to pass the current crosswise that is, at an angle to the ferrous parts.

The container comprises an outer box or shell 15 usually of cast iron or other suitable material, a lining 1 of refractory material which preferably consists of sections or bricks arranged end to end and assembled 110 within a sheet metal holder 16 which is removable from the shell 15, electrodes 2, 3 on opposite sides of the container and embedded in the sections of the lining 1, a cover for the container, and means for compressing the material in the container.

Usually, the shell 15 is formed with spacing ribs 17 on its inner face against the ends of which the outer face of the casing 16 abuts, the ribs forming an air space for 120 preventing loss of heat to the shell 15. A plurality of electrodes 2, 3 are arranged on opposite sides, of the container, each of which includes a head 18 located in a socket 19 in the inner face of a section or brick of 125 the lining 1, and a stem 20 extending through the brick, the holder 16 and the box or shell 1 to the outside thereof, where con-

- nection is made with an electric circuit. The stem 20 is connected to the head 18 by means of nuts 21, 22 screwing on the stem against the front and rear sides of the head
- 5 18. The contiguous or adjacent electrodes on each side of the container are connected by a pair of inductances 23 having like ends connected to the outer ends of the stems 20 of contiguous electrodes and having their
- 10 other ends connected to a feed wire 24. The inductances serve as means to distribute the current between opposite electrodes irrespective of the resistance or conductivity of the carbonizing material. Suitable switches may be arranged as at 25 to cut out electrodes in the event only a portion of the container is to be utilized and heated or if excess heat is generated in any part thereof.
- 15 26 is the cover for the container, the cover being clamped in position on the container in any suitable manner as by bolts passing through slotted lugs 27, 28 on the container and on the cover. The means associated with
- 20 the cover for compressing the carbonizing material comprises a plunger 29, and means as screws 30 threading through the cover and having hand wheels 31 at their upper ends.
- 25 30 The plunger 29 consist of a frame 32 which is connected directly to the threaded stems, and a plurality of sections 33 of refractory material detachably secured to the frame.
- 30 35 In operation, the articles are laid in the container between the electrodes and the carbonizing material packed around articles, and when the current is turned on it passes through the carbonizing material and cross-wise through the articles being treated.
- 35 The apparatus shown in Fig. 3 comprises a laminated core 10 surrounded by energizing coils 11 connected in an alternating current circuit, and containers 12 surrounding a portion of the core. The containers are of refractory and nonconductive material, are lined with graphite cylinders or rings and may comprise sub-divisions or sections 35. The core is substantially horseshoe shape
- 40 50 and is provided with a removable section 36 at the ends of the horseshoe for facilitating the arrangement of circular articles on the side bars of the core passing through the container. The articles are placed in the
- 55 60 container or the sections or compartments thereof after the core has been removed. Thereafter, the core is replaced, the opposite side bars thereof passing through the openings in the circular articles.
- 65 70 The carbonizing material is packed around the articles within the container and subjected to mechanical pressure. However, it is not essential that the articles encircle the core as they may be satisfactorily treated within the container even though they do

not encircle the core. In the operation of this apparatus the magnetic flux passing through the core induces a secondary current in the packing material and the graphite cylinders or rings and also in the articles themselves, and this current generates a high temperature in the packing material which effects the carbonizing. In some cases the carbonizing material or pellets may be entirely eliminated, the parts to be treated lying directly on the concentric graphite rings distributed through the container. Hence, a current is passing through the articles at the time they are being carbonized.

Our process is particularly advantageous in that the carbonizing material and articles therein can be brought to the required temperature in a few minutes, and it is necessary to maintain this temperature but a few minutes, as compared with hours by other processes, and furthermore, the degree of carbonization or the depth to which carbonization occurs in the articles can be regulated by turning off the current through the apparatus at any desired time.

We have determined by photo-micrography that a case formed by our process during a predetermined time, consists of pearlite of greater depth and contains less cementite than a case obtained by prior processes. For example, we obtain by our process a case of a given depth of pearlite in about one-third the time that this can be obtained by the older method. Furthermore, due to the fact that our process requires a relatively short time, the parts treated thereby can be quenched in a suitable cooling medium directly from the carbonizer, thus dispensing with the reheating of the parts for the purpose of refining the core.

What we claim is:

1. The process of carbonizing articles consisting in surrounding the article with a non fusible carbonizing material and quickly raising the temperature of such material, maintaining the same at a predetermined temperature for a certain length of time, and simultaneously passing an electric current through the articles and the material between electrodes spaced apart from the articles by the carbonizing material.

2. The process of carbonizing articles, the same consisting in surrounding the article with carbonizing material, subjecting said material to substantial mechanical pressure and then quickly raising the temperature of the packed material and maintaining the same at a predetermined temperature.

3. The process of carbonizing articles, the same consisting in surrounding the article with carbonizing material subjecting the material to substantial mechanical pressure to make the mass a conductor as a whole, and simultaneously applying an electric

- current to the mass of carbonizing material.
4. The process of carbonizing articles, the same consisting in surrounding the article with carbonizing material and quickly raising the temperature of such material by causing an electric current to pass therethrough between electrodes separated from the article by the carbonizing material.
- 10 5. The process of carbonizing articles, the same consisting in surrounding the article with carbonizing material and quickly raising the temperature of such material above the critical point by passing an electric current through the material between electrodes separated from the articles by the material surrounding the article.
- 15 6. The process of carbonizing the articles, the same consisting of surrounding the article with carbonizing material and quickly raising the temperature of such material to 1600° to 1800° F. more or less by generating heat in such articles by means of an electric current passing through the carbonizing material and the article from electrodes separated from the article by the carbonizing material.
- 20 7. An apparatus for carbonizing articles comprising a container having a lining of refractory material, electrodes exposed on the inner surface of the lining of each of
- 25
- 30
- two opposing sides of the container, feed wires and means connecting the feed wires and contiguous electrodes on each side of the container to distribute the current between opposite electrodes irrespective of the resistance or conductivity of the carbonizing material, substantially as and for the purpose described.
- 35 8. An apparatus for carbonizing articles comprising a container having a lining of refractory material, and electrodes exposed on the inner surface of the lining on opposite sides of the container, contiguous electrodes on each side being connected together by inductances connected at like ends to contiguous electrodes and at their other ends to a source of electrical energy supplying an alternating current, substantially as and for the purpose specified.
- 40
- 45
- 50
- 55
- In testimony whereof the applicants WILBUR and MURPHY have signed their names at Rochester, in the county of Monroe, and State of New York, this 16<sup>th</sup> day of June, 1917, and the applicant CANNON, at Syracuse, in the county of Onondaga, and State of New York, this 20th day of June, 1917.

MERRITT D. WILBUR.  
FRANCIS P. CANNON.  
THOMAS J. MURPHY.